

1

2,753,304

## LUBRICATING COMPOSITION

Gilbert H. Orozco, Euclid, Ohio, assignor to Pennsylvania Salt Manufacturing Co., Philadelphia, Pa., a corporation of Pennsylvania

No Drawing. Application September 26, 1955,  
Serial No. 536,786

15 Claims. (Cl. 252—18)

This invention relates to an improved lubricating composition for forming on metal stock, to be drawn or otherwise formed, a dry, homogeneous, self-adherent and tenacious lubricating and protective coating and particularly to an improved lubricating composition of which the principal lubricating ingredients are water-soluble soaps and one or more water-soluble inorganic water-liberating and glass-forming materials, of which all, or a major part, is an alkali metal borate.

The present invention also is an improvement on the composition disclosed in U. S. Letters Patent No. 2,530,837, issued to Orozco and Hendricks on November 21, 1950, and Reissue No. 23,184, issued to Roland A. Whitbeck on December 20, 1949.

The present improved composition relates to the type of lubricant commonly referred to as "dry lubricant" which is applied as an aqueous solution to the metal stock by dipping, spraying, or similar operation, and caused, or permitted, to dry thereon so as to form on the stock a dry, homogeneous, self-adherent, and tenacious protective and lubricating film as a result of which the dry coated stock can be subjected to pressure die forming operations and the like without the addition of other lubricating and cooling agents. As disclosed in the above-enumerated patents, compositions comprising water-soluble soap and one or more water-soluble, inorganic, water-liberating and glass-forming materials provide an effective coating for the metal stock during the desired drawing operations. Such compositions are generally used on large production lines in which many pieces of stock are continuously passing through the aqueous solutions to receive the coating. Some difficulty has occurred in this mass method of coating in that the organic and inorganic materials tend to draw out of the bath unevenly. This is objectionable since the ratio of organic to inorganic material will continuously change with the resulting coated stock possessing a coating that may contain a ratio of ingredients that is undesirable.

It is impractical to attempt to adjust or correct the bath for this constant change of ratio of ingredients due to the fact that the coating operation is continuous. Such an adjustment would require the taking of a sample of the bath and a resulting analysis thereof to determine the ratio of the ingredients. This procedure would be lengthy and by the time it would be completed, a large number of pieces of stock would have been passed through the bath with a possible further changing of the ratio of the ingredients. Similarly, the shutting down of the production line to take the sample and resulting analysis thereof would be economically unfeasible. Moreover, the maintenance of the bath at a constant ratio of organic to inorganic material usually is beyond the skill of the ordinary workman.

It has been found that by the addition of a coupling agent, or coupling and plasticizing agent, to the composition the aqueous solution thereof draws out uni-

2

formly, thus maintaining a uniform ratio of organic to inorganic material both in the bath and on the coated stock. The coupler alone has a marked effect upon maintenance of uniformity of the draw out of the bath and this is further enhanced by the presence in the bath of a plasticizer either as a separate material or in the form of a combined coupling and plasticizing material. In addition, and as a secondary effect, not only is the resultant coat on the stock more uniform in the ratio of organic to inorganic material, but it also appears to have a better consistency resulting in a more uniform drawing operation. Moreover, as a result of the use of this improved composition, the initial bath as used up can be increased from time to time merely by adding more of the original composition and a proportional amount of water so that the danger of changing the ratio of organic to inorganic material is eliminated.

The coupling agent, or combined coupling and plasticizing agent, or mixture of individual coupling and individual plasticizing agents, are added primarily to maintain the bath in uniform condition as the bath is drawn out or used up due to its application to the stock by dipping, spraying, and the like. Without the coupler or combined coupler and plasticizer the ratios of organic to inorganic material in the bath changes continuously during the application of the bath to the stock and it is very difficult to maintain a relatively constant ratio of organic to inorganic material in the bath by adding one or the other and proportionate amounts of water. The more equal draw out of the bath as a result of using a coupler or combined plasticizer and coupler appears to be due to a combined chemical and physical effect and the reduction of interfacial tension. The plasticizing effect apparently increases the adherence and pliability and coating which is beneficial in preventing dislodgment of the coating in initial stages of the draw in the dies. Instead, the plasticized coating will remain in place on the stock during operation of the die and thus will be carried into the proper place between the working faces of the die and stock. The plasticizing effect also assists in effecting uniform draw out of the bath. Again it eliminates the tendency of the coating to rub off as the stock drags across the cavity edges near the entrance of the female die.

45 The composition of the present invention comprises water-soluble high titre soap of which the melting point of the fatty acid content is at least about 36° C. or more and, in addition thereto, a larger amount of an alkali metal borate, in combination with a small amount of water-soluble coupling material and preferably both coupling and plasticizing material which may be a combined coupler and plasticizer or may be a mixture of a separate coupler and a separate plasticizer. If the composition is to be one to perform stepwise lubrication as set forth 50 in the above-identified Orozco and Hendricks patent, one or more other water-soluble, inorganic, water-liberating and glass-forming compounds, preferably alkali metal salts may be substituted for part of the borate though the total of such additional compounds should be maintained 55 at less than the total amount of borax.

While as indicated above and in the patents hereinbefore enumerated, the preferred water-soluble soaps to be employed in the formulation of compositions and in accordance with the present invention are high titre soaps, and particularly high titre soaps in which the mixed saponifiable fatty acid content thereof possesses a melting point of at least about 36° C., it is to be understood 65 that any water-soluble soaps that will provide the desired lubricity and will permit the formation of the necessary dry homogeneous coating of the completed composition without material moisture pick-up can be employed.

Therefore, water-soluble soaps in which the melting point of the mixed fatty acid content thereof is above that of normal room temperature of about 25° C. can in many metal working operations be employed satisfactorily, since such soaps impart the required properties to the completed composition.

Broadly stated the composition of the present invention comprises, by dry weight, the following:

|                                                                                                                                 | Range, parts       | Preferred, parts |
|---------------------------------------------------------------------------------------------------------------------------------|--------------------|------------------|
| Water-soluble high titre soap having a melting point of at least about 36° C.                                                   | 10 to 30           | 20               |
| Water-soluble, inorganic, water-liberating and glass-forming material of which all, or a major part, is an alkali metal borate. | 70 to 90<br>½ to 5 | 80               |
| Coupling and plasticizing material.                                                                                             |                    |                  |

As hereinbefore indicated, the agent to impart the coupling and plasticizing properties to the composition may be in the form of a single compound having both these characteristics or a separate coupler and a separate plasticizing agent may be employed. When separate agents are used, the coupler and plasticizer are employed in the ratio of about 4 parts of plasticizer to about 1 part coupler. The total amount of the two agents will be used within the range above set forth. In determining the ratio of separate couplers and plasticizers to each other to provide essentially the equivalent of a combined plasticizer and coupler, it is to be noted that the combined plasticizer and coupler is about 20% coupler and about 80% plasticizer, this being about 1 to 4 ratio of coupling effect to plasticizing effect. However, separate couplers are usually 100% couplers whereas separate plasticizers have about the same plasticizing effect as a combined plasticizer and coupler. Therefore, when separate coupling and separate plasticizing agents are used, the separate plasticizer is about  $\frac{1}{3}$  of the total of the two with the coupler being about  $\frac{1}{2}$  of the total.

The active lubricating ingredients of the composition and their functions when applied to the stock are clearly set forth in detail in the Orozco and Hendricks and Whiback patents hereinbefore identified. These patents give in detail the particular ingredients to be employed as well as the manner in which the particular proportions may be varied for the most economical and efficient operation relative to the particular draw. Generally, the high titre soap employed is one having a melting point of at least about 36° C. However, there are a great many high titre soaps having melting points well above 36° C. such as, for example, hydrogenated palm oil soap, hydrogenated tallow soap, stearin flux soap, "triple-pressed" tallow soap, cocoa butter soap, coaceric soap, Japanic soap, and borneo tallow soap, etc. The preferred soaps are tallow soap or palm oil soap having a melting point of at least about 36° C. or more, or any high titre soap having a melting point ranging from about 36° C. up. A titre of at least 41° C. is preferred for heavy draws. It is to be understood that a single soap may be used or it may be admixed with one or more other and additional soaps.

As indicated in the above patents, the water-soluble, inorganic, water-liberating, and glass-forming materials may be in the form of a single compound, this single compound being an alkali metal borate and preferably borax. That is to say, for many types of drawing operations, the alkali metal borate will be the sole inorganic lubricating ingredient. However, when stepwise lubrication is required as described in detail in the Orozco patent, one or more inorganic, water-soluble, water-liberating and glass-forming materials will be used. In general, these additional inorganic materials will be alkali metal salts such as, for example, sodium (mono-, di-, and tri-) phos-

phate, potassium (mono-, di-, and tri-), sodium carbonate, potassium carbonate, boric (ortho, meta and pyro) acid, sodium silicate, potassium silicate, etc.

As hereinbefore indicated, it is preferred to employ a single compound having both coupling and plasticizing properties in the blended composition. An illustrative class of materials possessing this dual function are sulfonated animal and vegetable oils and sulfonated unsaturated fatty acid derivatives thereof. Sulfonated mineral oil compounds in most circumstances are of no utility due to their inability to be effectively incorporated in the composition when in solution, although salts of sulfonated mineral oil derivatives, such as, for example, mahogany soaps, can be employed in the composition since this particular class of materials may be incorporated into the ultimate composition with little difficulty.

Illustrative examples of sulfonated vegetable oils which may be employed are as follows: castor, palm, palm kernel, olive rape seed, mustard seed, tea seed, sun flower seed, and coconut.

Among the sulfonated animal oils and fats that may be used are tallow, neat's-foot oil, lard oil, cod, herring, and whale oils, sperm, wool grease, oleic acid, ricinoleic, linoleic, etc.

Of the foregoing compounds possessing both coupling and plasticizing characteristics, the preferred material is a sulfonated vegetable oil with particular preference to be had for sulfonated castor oil. This compound is about 20% coupler and 80% plasticizer. If, for example, three parts of sulfonated castor oil is specified in a particular formula and a substitution is to be made therefor of a separate coupler and a separate plasticizer, the three parts would be made up of  $\frac{1}{2}$  part of coupler and  $2\frac{1}{2}$  parts of plasticizer.

When a separate coupler is to be employed, any surface active agent may be used. These compounds known as surface active agents are alkali metal salts of sulfates of long-chain alcohols, metal salts of sulfates of glycerides, alkylaryl metal sulfonates, pentaerythritol monoesters, esters of sulfosuccinic acid, sulfated aliphatic esters, and metal salts of sulfonated esters of aromatic hydrocarbons.

Specific examples of such surface active agents are sodium lauryl sulfate, sodium cetyl sulfate, sodium oleyl sulfate, potassium lauryl sulfate, sodium glycercyl monolaurate sulfate, dioctyl sodium sulfosuccinate, dicetyl potassium sulfosuccinate, sodium ketyl benzene sulfonate, sodium oleyl naphthalene sulfonate, and dihexyl sodium sulfosuccinate. For a complete list, including the above compounds, as well as fatty acid amides and esters known as surface active agents, reference is to be had to the article published in "Industrial and Engineering Chemistry," vol. 35, pp. 126-130, which gives a complete listing of commercially available surface active agents as well as identifying such agents chemically.

Of these surface active agents the alkali metal salts of sulfates of long-chain alcohols containing from about 8 to 18 carbon atoms are preferred. As a separate plasticizer to be employed in conjunction with one of the above-mentioned surface active agents, any of the vegetable and animal fats may be employed. That is to say, any of the oils which, when sulfonated, can be used as combined couplers and plasticizers may, if emulsified, but not sulfonated, be used as a plasticizer only. A rather detailed list of such oils is given hereinbefore and, if unsulfonated, may be used as the plasticizer.

Other plasticizers may be saponified oxygenated petroleum derivatives, water-soluble glycols, amorphous or microcrystalline waxes, etc. may be used. Of these materials, animal wool fat and rape seed oil are preferred.

Having described in detail the ingredients to be employed in formulating the composition of the present invention, it therefore becomes convenient to give a number of illustrative working examples of finished compositions which illustrate the present invention. In the following examples, the ratios given are by weight.

2,753,304

5

## Example 1

|                       | Parts |
|-----------------------|-------|
| Tallow soap           | 15    |
| Borax                 | 83    |
| Sulfonated castor oil | 2     |

## Example 2

|                       |    |
|-----------------------|----|
| Palm oil soap         | 6  |
| Tallow soap           | 10 |
| Borax                 | 82 |
| Sulfonated castor oil | 2  |

## Example 3

|                       |      |
|-----------------------|------|
| Palm oil soap         | 19.5 |
| Borax                 | 80   |
| Sulfonated castor oil | .5   |

## Example 4

|                       |      |
|-----------------------|------|
| Palm oil soap         | 15   |
| Borax                 | 82.5 |
| Sulfonated oleic acid | 2.5  |

## Example 5

|                     |      |
|---------------------|------|
| Tallow soap         | 20.5 |
| Borax               | 78   |
| Sulfonated corn oil | 1.5  |

## Example 6

|                          |    |
|--------------------------|----|
| Palm oil soap            | 22 |
| Borax                    | 74 |
| Sulfonated castor oil    |    |
| Sulfonated rape seed oil | 4  |

## Example 7

|                     |      |
|---------------------|------|
| Tallow soap         | 22.5 |
| Borax               | 73   |
| Sulfonated corn oil |      |
| Sulfonated palm oil | 4.5  |

## Example 8

|                      |      |
|----------------------|------|
| Palm oil soap        |      |
| Tallow soap          | 19   |
| Borax                | 80.5 |
| Sulfonated olive oil | .5   |

## Example 9

|                       |    |
|-----------------------|----|
| Tallow soap           | 22 |
| Borax                 | 75 |
| Sulfonated castor oil | 3  |

## Example 10

|                       |    |
|-----------------------|----|
| Palm oil soap         | 17 |
| Borax                 | 78 |
| Sulfonated castor oil | 5  |

## Example 11

|                            |      |
|----------------------------|------|
| Palm oil soap              | 17   |
| Potassium borate           | 79.5 |
| Sulfonated cotton seed oil | 3.5  |

## Example 12

|                            |    |
|----------------------------|----|
| Tallow soap                | 15 |
| Potassium borate           |    |
| Lithium borate             | 84 |
| Sulfonated cotton seed oil | 1  |

## Example 13

|                            |      |
|----------------------------|------|
| Tallow soap                | 15.5 |
| Lithium borate             | 84   |
| Sulfonated palm kernel oil | .5   |

6

## Example 14

|                       | Parts |
|-----------------------|-------|
| Stearin flux soap     | 22    |
| Borax                 | 77    |
| Sulfonated castor oil | 1     |

## Example 15

|                          |      |
|--------------------------|------|
| Hydrogenated tallow soap | 19   |
| Borax                    | 78.5 |
| Sulfonated coconut oil   | 2.5  |

## Example 16

|                             |    |
|-----------------------------|----|
| Hydrogenated palm oil soap  | 24 |
| Borax                       | 73 |
| Sulfonated coconut oil      |    |
| Sulfonated mustard seed oil | 3  |

## Example 17

|                              |    |
|------------------------------|----|
| "Triple-pressed" tallow soap |    |
| Hydrogenated palm oil soap   | 20 |
| Potassium borate             | 75 |
| Sulfonated tallow oil        | 5  |

## Example 18

|                     |      |
|---------------------|------|
| Cocoa butter soap   | 19.5 |
| Potassium borate    | 80   |
| Sulfonated lard oil | .5   |

## Example 19

|                       |    |
|-----------------------|----|
| Stearin flux soap     | 27 |
| Lithium borate        | 72 |
| Sulfonated tallow oil | 1  |

## Example 20

|                       |      |
|-----------------------|------|
| Coaceric soap         | 16   |
| Borax                 | 82.5 |
| Sulfonated castor oil | 1.5  |

## Example 21

|                  |      |
|------------------|------|
| Japanic soap     | 19   |
| Potassium borate |      |
| Borax            | 77.5 |

## Example 22

|                        |    |
|------------------------|----|
| Borneo tallow soap     | 21 |
| Borax                  |    |
| Lithium borate         | 75 |
| Sulfonated herring oil | 4  |

## Example 23

|                      |    |
|----------------------|----|
| Stearic acid soap    | 20 |
| Borax                | 79 |
| Sulfonated sperm oil | 1  |

## Example 24

|                      |    |
|----------------------|----|
| Stearin flux soap    |    |
| Stearic acid soap    | 22 |
| Borax                |    |
| Lithium borate       | 74 |
| Sulfonated whale oil |    |
| Sulfonated sperm oil | 4  |

## Example 25

|                                |    |
|--------------------------------|----|
| Borneo tallow soap             |    |
| "Triple-pressed" palm oil soap | 18 |
| Borax                          | 80 |
| Sulfonated herring oil         | 2  |

## Example 26

|                       |    |
|-----------------------|----|
| Stearin flux soap     | 21 |
| Borax                 | 78 |
| Sulfonated castor oil | 1  |

## 7 Example 27

|                      | Parts |
|----------------------|-------|
| Tallow soap          | 22    |
| Borax                | 55    |
| Potassium carbonate  | 21    |
| Sulfonated sperm oil | 2     |

## Example 28

|                       |      |
|-----------------------|------|
| Tallow soap           | 19.5 |
| Stearin flux soap     |      |
| Boric acid            | 70   |
| Borax                 | 10   |
| Sulfonated oleic acid | .5   |

## Example 29

|                       |      |
|-----------------------|------|
| Palm oil soap         | 15   |
| Borax                 | 51   |
| Trisodium phosphate   | 15   |
| Potassium carbonate   | 18.5 |
| Sulfonated castor oil | .5   |

## Example 30

|                            |    |
|----------------------------|----|
| Cocoa butter soap          | 15 |
| Lithium borate             | 83 |
| Sulfonated ricinoleic acid | 2  |

## Example 31

|                          |      |
|--------------------------|------|
| Japanic soap             | 17   |
| Borax                    | 51.5 |
| Sodium silicate          | 10   |
| Boric acid               | 8    |
| Sodium phosphate         | 12   |
| Sulfonated oleic acid    |      |
| Sulfonated linoleic acid | 1.5  |

## Example 32

|                       |    |
|-----------------------|----|
| Palm oil soap         | 20 |
| Borax                 | 57 |
| Sodium silicate       | 5  |
| Potassium carbonate   | 15 |
| Sulfonated castor oil | .3 |

## Example 33

|                       |    |
|-----------------------|----|
| Tallow soap           | 15 |
| Borax                 | 45 |
| Sodium carbonate      | 15 |
| Sodium silicate       | 10 |
| Trisodium phosphate   | 12 |
| Sulfonated castor oil | 3  |

## Example 34

|                       |    |
|-----------------------|----|
| Tallow soap           | 15 |
| Borax                 | 40 |
| Boric acid            | 20 |
| Potassium carbonate   | 22 |
| Sulfonated castor oil | 2  |

## Example 35

|                     |    |
|---------------------|----|
| Palm oil soap       | 20 |
| Borax               | 39 |
| Disodium phosphate  | 15 |
| Boric acid          | 10 |
| Potassium carbonate | 12 |
| Mahogany soap       | 4  |

## Example 36

|                     |    |
|---------------------|----|
| Palm oil soap       | 22 |
| Tallow soap         |    |
| Borax               | 55 |
| Sodium silicate     | 5  |
| Boric acid          | 8  |
| Potassium carbonate | 8  |
| Sulfonated corn oil | 2  |

## Example 37

|                              |      |
|------------------------------|------|
| "Triple-pressed" tallow soap | 17.5 |
| Borax                        | 44   |
| Trisodium phosphate          | 20   |
| Potassium carbonate          | 15   |
| Sulfonated sperm oil         | 3.5  |

## 8 Example 38

|                       | Parts |
|-----------------------|-------|
| Japanic soap          | 20    |
| Potassium borate      | 65    |
| 5 Sodium carbonate    | 5     |
| Potassium phosphate   | 5     |
| Boric acid            | 4     |
| Mahogany soap         |       |
| Sulfonated oleic acid | 1     |

## Example 39

|                       |    |
|-----------------------|----|
| Tallow soap           | 12 |
| Borax                 | 86 |
| Sodium lauryl sulfate |    |
| Cottonseed oil        | 2  |

## Example 40

|                      |    |
|----------------------|----|
| Palm oil soap        | 20 |
| Borax                | 77 |
| Sodium octyl sulfate |    |
| 20 Sperm oil         | 3  |

## Example 41

|                                        |    |
|----------------------------------------|----|
| Palm oil soap                          | 16 |
| Tallow soap                            |    |
| Potassium borate                       | 80 |
| 25 Sodium glyceryl monolaurate sulfate | 4  |
| Rape seed oil                          |    |

## Example 42

|                               |    |
|-------------------------------|----|
| Stearin flux soap             | 24 |
| 30 Potassium borate           |    |
| Lithium borate                | 75 |
| Diethyl sodium sulfosuccinate |    |
| Animal wool fat               | 1  |

## Example 43

|                              |    |
|------------------------------|----|
| Hydrogenated tallow soap     | 18 |
| Borax                        | 77 |
| Pentaerythritol monostearate |    |
| 50 Corn oil                  | 5  |

## Example 44

|                                |      |
|--------------------------------|------|
| Hydrogenated palm oil soap     | 15   |
| Borax                          |      |
| Potassium borate               | 83.5 |
| 45 Pentaerythritol monolaurate | 1.5  |
| Palm oil                       |      |

## Example 45

|                                       |    |
|---------------------------------------|----|
| Cocoa butter soap                     | 17 |
| Borax                                 | 80 |
| Sodium $\beta$ -oleylethane sulfonate |    |
| 50 Tallow oil                         | 3  |

## Example 46

|                              |      |
|------------------------------|------|
| Coaceric soap                | 14.5 |
| Potassium borate             | 82   |
| 55 Sodium ricinoleyl sulfate |      |
| Coconut oil                  | 3.5  |

## Example 47

|                                |      |
|--------------------------------|------|
| Borneo tallow soap             | 13.5 |
| Lithium borate                 | 86   |
| 60 Neat's-foot oil             |      |
| Sodium ketyl benzene sulfonate | .5   |

## Example 48

|                       |    |
|-----------------------|----|
| Stearin flux soap     | 20 |
| 65 Stearic acid soap  |    |
| Borax                 | 77 |
| Sodium lauryl sulfate |    |
| Palm kernel oil       | 3  |

## Example 49

|                         |    |
|-------------------------|----|
| Borneo tallow soap      | 11 |
| Japanic soap            |    |
| Lithium borate          | 87 |
| Potassium cetyl sulfate |    |
| 75 Lecithin             | 2  |

## Example 50

|                                   | Parts |
|-----------------------------------|-------|
| Tallow soap                       | 18    |
| Coaceric soap                     | 18    |
| Borax                             | 81    |
| Potassium borate                  | 5     |
| Dilauryl potassium sulfosuccinate | 1     |
| Rape seed oil                     | 1     |

## Example 51

|                                    | Parts |
|------------------------------------|-------|
| Japanic soap                       | 13    |
| Palm oil soap                      | 13    |
| Borax                              | 65.5  |
| Boric acid                         | 8     |
| Potassium carbonate                | 10    |
| Sodium octyl naphthalene sulfonate | 3.5   |
| Wool fat                           | 1     |

## Example 52

|                       | Parts |
|-----------------------|-------|
| Palm oil soap         | 15    |
| Borax                 | 40    |
| Boric acid            | 18    |
| Potassium carbonate   | 24    |
| Rape seed oil         | 3     |
| Sodium lauryl sulfate | 1     |

## Example 53

|                              | Parts |
|------------------------------|-------|
| Tallow soap                  | 22.5  |
| Borax                        | 60    |
| Trisodium phosphate          | 15    |
| Pentaerythritol monostearate | 1     |
| Herring oil                  | 2.5   |

## Example 54

|                                       | Parts |
|---------------------------------------|-------|
| Palm oil soap                         | 20    |
| Tallow soap                           | 20    |
| Borax                                 | 52    |
| Sodium silicate                       | 8     |
| Disodium phosphate                    | 10    |
| Boric acid                            | 5     |
| Sodium $\beta$ -oleylethane sulfonate | 5     |
| Cottonseed oil                        | 1     |

## Example 55

|                       | Parts |
|-----------------------|-------|
| Cocoa butter soap     | 15    |
| Potassium borate      | 48.5  |
| Sodium carbonate      | 15    |
| Potassium phosphate   | 15    |
| Sodium silicate       | 5     |
| Sodium lauryl sulfate | 1.5   |
| Rape seed oil         | 1     |

## Example 56

|                           | Parts |
|---------------------------|-------|
| Palm oil soap             | 18    |
| Borax                     | 65    |
| Boric acid                | 15    |
| Sodium ricinoleyl sulfate | 2     |
| Palm oil                  | 1     |

## Example 57

|                             | Parts |
|-----------------------------|-------|
| Tallow soap                 | 22    |
| Borax                       | 55    |
| Trisodium phosphate         | 12    |
| Potassium carbonate         | 8     |
| Pentaerythritol monolaurate | 3     |
| Cod fish oil                | 1     |

## Example 58

|                      | Parts |
|----------------------|-------|
| Japanic soap         | 15    |
| Tallow soap          | 15    |
| Borax                | 50    |
| Boric acid           | 6     |
| Potassium carbonate  | 20    |
| Sodium silicate      | 5     |
| Sodium octyl sulfate | 4     |
| Whale oil            | 1     |

## Example 59

|                               | Parts |
|-------------------------------|-------|
| Palm oil soap                 | 24.5  |
| Borax                         | 53    |
| Disodium phosphate            | 8     |
| Boric acid                    | 5     |
| Sodium carbonate              | 8     |
| Diethyl sodium sulfosuccinate | 1.5   |
| Rape seed oil                 | 1     |

## Example 60

|                                     | Parts |
|-------------------------------------|-------|
| Palm oil soap                       | 13    |
| Tallow soap                         | 60    |
| Potassium borate                    | 15    |
| Trisodium phosphate                 | 15    |
| Potassium carbonate                 | 6.5   |
| Sodium silicate                     | 5     |
| Sodium glyceryl monolaurate sulfate | .5    |
| Lecithin                            | .5    |

20 The composition is dissolved in water in an amount ranging from one ounce of the dry mix to two pounds of the dry mix per gallon of water, depending upon the particular characteristics of the stock, dies and draw. The resultant solution is applied to the stock to be drawn in any suitable manner such, for example, as by dipping, after which the coated stock is permitted to dry or is dried by the application of heat so as to form on the stock a dry, homogeneous, self-adherent, lubricating film which is very tenacious and which remains on the stock under normal storage conditions, both protecting it during storage and providing all the lubricant that is necessary when the stock is subsequently drawn.

35 An increase in the soap content above the lower limit provides better lubrication at lower temperatures and pressures whereas an increase in the borate content or mixture of borate and other inorganic materials provides better lubrication at the higher pressures and temperatures. On the other hand, an excess of soap over that required for a particular draw may result in building up of a relatively hard putty-like mass on the working surfaces of the dies with resultant scoring and marring of the stock and interference with the mechanical operations of the dies, ejectors, and operating mechanisms. An excess of soap above the upper limit recited results in a tacky coating or film having low or little adherence to the stock.

40 An excess of the borate or mixture for a particular draw produces a film which is apt to flake off, or fail to operate properly in that the stock, because of lack of lubrication initially, becomes scored before a high enough pressure and temperature are reached to render the borate fully operative. Moreover, an excess of borate above the upper limit recited results in coating which is dusty, or causes a dusty condition in the dies, and which has insufficient plasticity and adherence.

45 Many coexisting factors must be considered in choosing the proportions of ingredients in the dry mix and the density of the solution for a given draw. These include, for example, the type of metal, its thickness, surface condition, ductility and other physical characteristics; the type of dies, die tolerance or clearance and surface or finish; and the depth and complexity of the draw; the speed of the presses and length of stroke.

50 In general, for stock having a high polish or mirror finish and for stainless steels a very thin coating is required as the adherence of thinner films is greater than that of the thicker films. Deep draws and resultant high pressures and temperatures usually indicate the higher borate to soap ratio than lighter draws and lower temperatures and pressures. Rough surface stock requires a relatively thick coat in that the surface cavities of the stock as well as the surface projections should be well coated. New dies or dies with close clearance require a thinner film than older dies or dies with more clearance.

## 11

The thinnest coating consistent with proper lubrication is desirable.

Accordingly, for the thinnest films, such as used for highly polished or stainless steels, the dry mix is used in an amount of about two ounces per gallon of water. For the coarsest films, such as used for rough finished stock, the dry mix may be used in an amount as high as two pounds per gallon. A few trials with any particular stock of steel or other metal in the particular dies to be used will demonstrate the film thickness and ratio of ingredients that may be used for optimum results for the particular metal and draw.

By the term "consisting essentially of" as used herein in defining the coating composition or film, it is meant to define a composition or film containing the claimed ingredients, in the relative proportions stated as the possible and actual constituents of the composition or film, but it is not meant to exclude the presence of minor amounts of conventional compounds or ingredients, the use of which is common practice in the lubrication of metals during forming operations.

The present application is a continuation-in-part of my now abandoned co-pending application Serial No. 251,455, filed October 15, 1951, which, in turn, is a continuation of my now abandoned application Serial No. 53,376, filed October 7, 1948.

Having described the invention, I claim:

1. A coating material for admixture with water for coating a piece of blank metal stock in forming thereon a self-adherent dry homogeneous lubricating and protecting film consisting essentially of the following lubricating ingredients:

Parts  
Water-soluble, high titre soap having a melting point of at least about 36° C. 10 to 30  
Water-soluble, inorganic, water liberating and glass forming material of which at least a major part thereof is an alkali metal borate. 70 to 90  
Coupling and plasticizing material selected from the groups consisting of the following: 1/2 to 5

A. Combined coupling and plasticizing material in the form of at least one compound selected from the group consisting of sulfonated vegetable oils, sulfonated animal oils, and sulfonated unsaturated fatty acid derived from animal oil and vegetable oil; 45

B. Coupling and plasticizing material in the form of at least two compounds, at least one compound being selected from each of the following groups—

1. Coupling agent: Surface active, water-soluble, alkali metal salts of organic compounds containing a sulfo-group in the molecule;  
2. Plasticizing agent: Vegetable oils and animal oils.

2. A coating material in accordance with claim 1 wherein the coupling and plasticizing material is a sulfonated vegetable oil.

3. A coating material in accordance with claim 1 wherein the coupling and plasticizing material is a sulfonated animal oil.

4. A coating material in accordance with claim 1 wherein the coupling and plasticizing material is a sulfonated unsaturated fatty acid derived from animal oil and vegetable oil.

5. A coating material in accordance with claim 1 wherein the coupling and plasticizing material is sulfonated castor oil.

## 12

6. A coating material in accordance with claim 1 wherein the coupling and plasticizing material is sulfonated cottonseed oil.

7. A coating material in accordance with claim 1 wherein the coupling and plasticizing material is sulfonated corn oil.

8. A coating composition in accordance with claim 1 wherein the coupling agent is an alkali metal organic sulfate.

9. A coating composition in accordance with claim 1 wherein the coupling agent is an alkali metal organic sulfonate.

10. A coating composition in accordance with claim 1 wherein the coupling agent is an alkali metal salt of a sulfate of an aliphatic alcohol.

11. A coating composition in accordance with claim 1 wherein the coupling agent is sodium lauryl sulfate.

12. A coating composition in accordance with claim 1 wherein the coupling agent is sodium ketyl benzene sulfonate.

13. A coating composition in accordance with claim 1 wherein the coupling agent is dioctyl sodium sulfosuccinate.

14. A coating material for admixture with water for coating a piece of blank metal stock in forming thereon a self-adherent, dry, homogeneous lubricating and protecting film consisting essentially of the following ingredients by weight:

| Parts                                                                                  |
|----------------------------------------------------------------------------------------|
| Water-soluble high titre soap having a melting point of at least about 36° C. 10 to 30 |
| Borax 70 to 90                                                                         |
| Sulfonated castor oil 1/2 to 5                                                         |

15. A coating material for admixture with water for coating a piece of blank metal stock in forming thereon a self-adherent dry homogeneous lubricating and protecting film consisting essentially of the following lubricating ingredients:

| Parts                                                                                                                                            |
|--------------------------------------------------------------------------------------------------------------------------------------------------|
| A water-soluble soap 10 to 30                                                                                                                    |
| Water-soluble, inorganic, water liberating and glass forming material of which at least a major part thereof is an alkali metal borate. 70 to 90 |
| Coupling and plasticizing material selected from the groups consisting of the following: 1/2 to 5                                                |

A. Combined coupling and plasticizing material in the form of at least one compound selected from the group consisting of sulfonated vegetable oils, sulfonated animal oils, and sulfonated unsaturated fatty acid derived from animal oil and vegetable oil;

B. Coupling and plasticizing material in the form of at least two compounds, at least one compound being selected from each of the following groups—

1. Coupling agent: Surface active, water-soluble alkali metal salts of organic compounds containing a sulfo-group in the molecule;  
2. Plasticizing agent: Vegetable oils and animal oils.

## References Cited in the file of this patent

## UNITED STATES PATENTS

|           |               |               |
|-----------|---------------|---------------|
| 2,252,385 | Orozco        | Aug. 12, 1941 |
| 2,326,387 | Nill          | Aug. 10, 1943 |
| 2,352,811 | Swenson       | July 4, 1944  |
| 2,578,586 | Orozco et al. | Dec. 11, 1951 |
| 2,609,594 | Whitbeck      | Sept. 9, 1952 |